

## UNITED STATES PATENT OFFICE

2,471,384

## FROTH FLOTATION OF SULFIDE ORES

Robert B. Booth, Springdale, and Roy A. Pickens,  
Stamford, Conn., assignors to American Cyanamid Company, New York, N. Y., a corporation of Maine

No Drawing. Application May 16, 1946,  
Serial No. 670,313

3 Claims. (Cl. 209—167)

1

This invention relates to the beneficiation of metallic sulfide ores and in particular to the separation of one or more metal sulfide minerals each from the other and/or from other minerals or gangue, particularly slimy gangues. As such the present invention constitutes a continuation-in-part of our copending application, Serial No. 639,164, filed January 4, 1946.

The term "sulfide ores" as used herein is employed in the broad sense to describe those ores of whose mineral values are mainly in the form of sulfide minerals and also to describe ores whose values may be in the form of sulfide minerals associated with other values in the form of native metal and oxide or oxidized minerals. For example, copper ores frequently contain a portion of their values as sulfides, chalcocite, covellite, and chalcopyrite associated with pyrite, molybdenite, native copper, cuprite, bornite, azurite, malachite and chrysocolla. Similarly lead sulfide ores frequently contain galena associated with cerrusite and anglesite, while zinc ores often contain sphalerite associated with willemite, smithsonite and calamine.

Beneficiation of metallic sulfide ores by froth flotation has come to be commonly accepted as almost a standardized procedure. The process is carried out in acid, neutral or alkaline circuits in the presence of a promoter and, usually, a frothing agent. Many materials have been suggested for use as promoters. The most widely accepted in use have come to be the xanthate and dithiophosphoric acids and dithiophosphate types. These have been found excellent and have achieved almost universal acceptance.

However, it must be realized that in such operations a relatively tremendous amount of feed is handled to obtain a relatively small amount of desirable mineral in the concentrate. Consequently the amount of valuable material left in the tailing is a highly important factor. Usually the more the mineral value content of the tailing can be reduced the more highly satisfactory the operation. In addition thereto, there is the problem of obtaining a high ratio of concentration. Usually this latter is of primary importance, the grade of concentrate being the most critical measure of the degree of success of the operation. At times, however, the freedom of the tailing from valuable mineral content may become equally if not more important.

The difficulty may be illustrated, for example, in the concentration of copper minerals from a typical feed containing other sulfides such as those of lead or zinc or both, gangue and secondary slimes. Using a good commercially available promoter, it is frequently possible to produce copper sulfide concentrates which may be of higher grade than the commercially acceptable minimum. It is ordinarily desirable to do so since premiums are usually paid based on the higher

content of copper mineral in the concentrate. Beyond a certain point, however, increasing the copper content of the concentrate is done at the expense of increasing the copper content of the tailing. A practical economic balance therefore must be made and subsequently followed as nearly as possible in which the degree of concentration and the copper content in the tailing are both considered in determining the optimum recovery.

Unfortunately, even good practice with the better promoters frequently will not permit reducing the copper content of the tailing to a point as low as is desired without producing a less than premium grade concentrate. This problem has faced the art for many years and many auxiliary agents have been suggested for modifying the action of the promoter during flotation, without fully accomplishing the desired results. It is therefore the principal object of the present invention to develop a surface-modifying agent for use in the beneficiation of sulfide ores which when properly used will enhance both the selectivity and the collecting power of the better of the presently available promoters. At the same time it is desirable that the modifying agent or agents be readily available, relatively inexpensive, easily used and capable, once their optimum use is determined, of reliably duplicating the desired result.

Surprisingly these desirable results are simply and easily obtained by using the proper amount of a suitable lignin sulfonate as the surface modifier for the mineral constituents of the flotation pulp. Although this type of reagent appears to have the effect of such a surface-modifying action on the minerals, the exact nature of its action is not wholly understood. Their action, however, is highly reliable. As shown in our above identified copending application, in the beneficiation of copper sulfide minerals, for example, they may be used to reduce the copper content of the tailing by as much as one-half.

In addition to this valuable property, in accordance with the present invention it has also been found that their surface-modifying effect is progressively selective. Thus, by the proper use it is perfectly feasible to progressively separate with a high degree of concentration first one sulfide mineral and then another. These practices are familiar in the art of treatment of mixed ores containing a plurality of valuable minerals. In the separation of one sulfide mineral from another the lignin sulfonates used in accordance with the present invention are selectively effective in each of the separation, appearing to enhance the collection of the desired fraction by the promoter while depressing the other sulfides and/or other undesirable mineral values and gangue.

2

The form in which the lignin sulfonate is used in the practice of the present invention is not necessarily critical in most cases. If desired it may be used in acid form. The amount used is not sufficient to markedly alter the pH of a neutral circuit. Therefore whether an acid form is fed to an acid or alkaline circuit makes little difference. Nor does it appreciably alter the process if an alkaline lignin sulfonate is added to either an acidic or alkaline circuit.

In general the alkali metal or alkaline earth metal lignin sulfonates including the ammonium salts are preferable because they are available commercially either in the form of solutions or as dry powders. The latter are easily shipped to the point of use, are readily soluble in water and may be fed without difficulty. The sodium, ammonium, calcium, barium and magnesium salts as well as mixtures thereof have been successfully used. Lignin sulfonates for use in the present invention may be either purposely synthesized, or commercially available products may be used. These latter, derived usually from the manufacture of pulp and paper, are often obtainable in highly purified condition. However, for the purpose of the present invention this is not essential. In many cases the degree of purity appears to be of concern only in so far as it effects the amount to be used. Since the crude products may be used, an inexpensive source of supply is readily available in the material recovered in the sulfate process for the manufacture of wood pulp. While the magnesium salt is useful as is the barium salt, they are generally found less satisfactory than the calcium, sodium or ammonium salts. Since the calcium salt is generally more readily available, it is perhaps to be preferred.

The amount of lignin sulfonate used will obviously vary with a number of factors. These will include such variables as the degree of purity of the lignin sulfonate, the nature of the ore, the amount of promoting reagent required, the temperature of the process water and many others. In general, only enough should be used to produce the desired surface-modifying action. For most operations this will be found to lie between about 0.01 to 0.30 lb./ton of feed.

At times or with some conditions as much as 0.50 lb./ton of ore may be required. In general, however, excessive amounts should be avoided. One of the features of the use of the lignin sulfonates as surface modifiers for this purpose is in its successful inhibition of the undesired minerals during the promotion and collection of the desired fraction. Moderate excesses of surface-modifying agent over the amount necessary to produce the desired selective depression have no particular effect on the process. However, larger excesses may be found to interfere with the promotion of the desired mineral and thus interfere with the desirable result obtained by the presence of smaller amounts. The upper limit then may be expressed generally as being somewhat less than that amount which depresses the values which it is desired to recover. It is quite surprising that this effective range of small amounts exists whereas the presence of excessive amounts may be harmful.

Because the action of the beneficiating reagents of the present invention is one of surface modification, they may be employed in any one of several ways. If equipment is available for the purpose, a conditioning operation with the surface modifier before carrying out the flotation is usually advantageous. It may even be further advan-

tageous in many cases to condition the flotation feed with the modifying agent before the promoter is added thereto. This is not difficult since the lignin sulfonate may be added during the grinding operation or in a pre-conditioning step using a simple mechanical agitator. The surface modifier may be added to the pulp along with the promoter. It may be used to direct addition to the flotation cell just prior to or even during flotation. In these various operations it may be used in dry form, as a paste, as aqueous dispersions or suspensions, or in aqueous solution. The latter is preferable in most cases because it simplifies control of the amounts fed, particularly of the small amounts used.

It is a feature of the present invention that it may be employed in any of several ways. It may be used to enable the production of concentrates of equal grade to those obtained by the practice of the prior art while obtaining these concentrates with higher recovery. On the other hand, if a premium on extremely high grade is available, it may be desirable to use the surface modifier to obtain recoveries approximating those obtainable by the practice of the prior art while increasing the grade to as high a degree as possible. Whichever of these two practices is to be followed will be a factor in determining the quantities of reagents used. This is true both with respect to the amount of promoter and with respect to the surface-modifying agent of the present invention.

The present invention will be described in detail in conjunction with the following examples which are meant to be illustrative only and not by way of limitation. All parts are by weight unless otherwise noted.

#### EXAMPLE 1

A copper ore from the southwestern part of the United States assaying approximately 1.20% Cu and containing pyrite, chalcocite, covellite, chalcopyrite, malachite, sphalerite, limonite, quartz, sericite, chlorite, biotite and carbonate was ground to about minus 65 mesh, conditioned at 22% solids with 0.064 lb./ton cresylic acid, 0.028 lb./ton of a 1:1 mixture of sodium diethyl and dissecondary butyl dithiophosphates, and varying amounts of lignin sulfonates, and then floated in a Fagergren flotation machine. The results of these tests are summarized in the following table:

Table I

| Lbs./ton | Lignins Reagent Type                   | Concentrate, percent Total Cu |        | Tailing, percent Total Cu, Assay |
|----------|----------------------------------------|-------------------------------|--------|----------------------------------|
|          |                                        | Assay                         | Recov. |                                  |
| 60       | No Lignin Sulfonate used.              | 15.81                         | 64.03  | 0.44                             |
|          | Purified Calcium Lignin Sulfonate..... | 10.00                         | 84.88  | 0.19                             |
|          | .....do.....                           | 14.82                         | 70.64  | 0.38                             |
|          | Crude Sodium Lignin Sulfonate.....     | 14.14                         | 72.40  | 0.355                            |
| 65       | .....do.....                           | 14.29                         | 68.02  | 0.40                             |
|          | Neutral Calcium Lignin Sulfonate.....  | 13.92                         | 73.10  | 0.345                            |
|          | .....do.....                           | 11.62                         | 77.83  | 0.28                             |
|          | Basic Calcium Lignin Sulfonate.....    | 11.05                         | 81.47  | 0.235                            |
| 70       | Acid Magnesium Lignin Sulfonate.....   | 15.60                         | 65.83  | 0.42                             |
|          | .....do.....                           | 17.12                         | 60.80  | 0.49                             |
|          | Neutral Sodium Lignin Sulfonate.....   | 14.97                         | 66.83  | 0.42                             |
|          | .....do.....                           | 14.97                         | 68.33  | 0.40                             |
| 75       | Neutral Ammonium Lignin Sulfonate..... | 12.88                         | 75.88  | 0.31                             |
|          | .....do.....                           | 11.00                         | 85.13  | 0.19                             |

## EXAMPLE 2

The primary slime portions of a copper ore from the southwestern United States, obtained by desliming the ore prior to leaching, were treated with 0.32 lb./ton crude calcium lignin sulfonate, 0.035 lb./ton potassium ethyl xanthate, 0.06 lb./ton pine oil, and 3.9 lb./ton lime and floated for 8 minutes. From a feed to flotation, assaying 1.04% Cu, of which about half was sulfide copper and about half non-sulfide copper, 85.4% of the copper was obtained as a concentrate assaying 17.8% Cu. The tailings assayed 0.16% Cu.

A similar treatment without the lignin sulfonate gave a recovery of 78.0% of the copper in a concentrate assaying 17.9% Cu. The tailing from this treatment assayed 0.24% Cu.

## EXAMPLE 3

A Tennessee zinc ore of about 3.2% Zn content was ground and conditioned with 0.5 lb./ton copper sulfate, 0.1 lb./ton American Cyanamid Company Sodium Aerofloat B, and 0.14 lb./ton pine oil, and then floated for 2 minutes. 0.04 lb./ton pine oil was then added and flotation continued for 2 minutes longer. Similar tests were conducted using 0.05 and 0.1 lb./ton of mono calcium lignin sulfonate. Metallurgical results were as follows:

Table II

| Lbs./Ton of Modifier | Concentrate, per cent Zn |        | Tailing, per cent Zn, Assay |
|----------------------|--------------------------|--------|-----------------------------|
|                      | Assay                    | Recov. |                             |
| None                 | 46.94                    | 91.65  | 0.284                       |
| 0.05                 | 48.35                    | 91.87  | 0.284                       |
| 0.10                 | 52.47                    | 91.37  | 0.298                       |

## EXAMPLE 4

A Tri-State lead ore, containing about 2.5%

40 The following metallurgical results were obtained:

Table IV

| Test | Lead Concentrate |       |             |       | Zinc Concentrate |       |             |       | Tailing Assay |             |
|------|------------------|-------|-------------|-------|------------------|-------|-------------|-------|---------------|-------------|
|      | Per Cent Pb      |       | Per Cent Zn |       | Per Cent Zn      |       | Per Cent Pb |       |               |             |
|      | Assay            | Dist. | Assay       | Dist. | Assay            | Dist. | Assay       | Dist. | Per Cent Pb   | Per Cent Zn |
| A    | 61.77            | 95.63 | 1.81        | 0.33  | 57.27            | 97.54 | 0.24        | 3.38  | 0.05          | 0.44        |
| B    | 66.03            | 98.00 | 1.96        | 0.39  | 56.86            | 97.43 | 0.059       | 1.23  | 0.036         | 0.48        |
| C    | 71.60            | 93.64 | 1.40        | 0.24  | 56.86            | 97.36 | 0.272       | 3.15  | 0.095         | 0.54        |
| D    | 71.00            | 95.88 | 1.97        | 0.32  | 59.60            | 97.24 | 0.14        | 1.85  | 0.06          | 0.52        |

Pb, was ground with 0.035 lb./ton sodium isopropyl xanthate and about 0.2 lb./ton creosote oil and after dilution to flotation density, about 22% solids, was conditioned with 0.04 lb./ton of a mixture of amyl alcohols, pentasol, for 0.5 minute in a laboratory Fagergren flotation machine. Flotation followed for 5 minutes. Similar tests were conducted using 0.05, 0.10, and 0.20 lb./ton calcium lignin sulfonate which was added to conditioning. Metallurgical results were as follows:

55

The lignin sulfonates may be used without cyanide in the separation of sulfides by flotation. The lead-zinc ore used in Example 5 was treated as described in that example except that the use of cyanide was omitted. The following tests were conducted using calcium lignin sulfonate in the first conditioning step only. In the first test no lignin sulfonate was used; in the second test 0.2 lb./ton of calcium lignin sulfonate was used. The metallurgical results are as follows:

Table V

| Lead Concentrate |       |             |       | Zinc Concentrate |       |             |       | Tailing, Assay |             |
|------------------|-------|-------------|-------|------------------|-------|-------------|-------|----------------|-------------|
| Percent Pb       |       | Per cent Zn |       | Per cent Zn      |       | Per cent Pb |       |                |             |
| Assay            | Dist. | Assay       | Dist. | Assay            | Dist. | Assay       | Dist. | Per cent Pb    | Per cent Zn |
| 59.88            | 96.72 | 3.14        | 0.64  | 59.11            | 96.61 | 0.06        | 0.77  | 0.07           | 0.61        |
| 58.81            | 95.44 | 0.88        | 0.18  | 59.05            | 96.54 | 0.25        | 3.18  | 0.04           | 0.74        |

## EXAMPLE 7

An African gold ore, assaying about 0.374-0.396 oz. Au/ton and containing chalcopyrite, bornite, pyrrhotite, quartz and sericite, was ground to minus 65 mesh and treated as follows:

1. Conditioned 5 minutes at 22% solids with 0.5 lb./ton crude calcium lignin sulfonate.

2. Conditioned 2 minutes longer with 0.3 lb./ton secondary butyl xanthate, 0.03 lb./ton of a 1:1 mixture of sodium ethyl and sec. butyl dithiophosphates, and 0.03 lb./ton pine oil.

3. Floated 10 minutes in a Fagergren flotation machine; after 5 minutes of flotation 0.05 lb./ton sec. butyl xanthate and 0.03 lb./ton pine oil were added and flotation continued 5 minutes longer.

A second test was conducted, which was similar in all details to the above-described test except that no lignin sulfonate was used.

The metallurgical results of both tests are given in the following table. It will be noted that marked improvements in the grade of the concentrate and ratio of concentration resulted in the test employing the lignin sulfonate. Losses of gold in the tailings were practically identical in both tests.

Table VI

| Lb./Ton Lig-nin Sulfonate | Feed Assay, Oz.Au/Ton | Concentrate             |                  |                     | Tailing Assay, Oz.Au/Ton |
|---------------------------|-----------------------|-------------------------|------------------|---------------------|--------------------------|
|                           |                       | Ratio of Concentra-tion | Assay, Oz.Au/Ton | Per cent Au. Recov. |                          |
| 0.5.....                  | 0.347                 | 22.1:1                  | 7.640            | 92.25               | 0.030                    |
| None.....                 | 0.398                 | 13.0:1                  | 4.810            | 93.43               | 0.028                    |

We claim:

1. In the beneficiation by froth flotation of a metallic sulfide mineral by means of a promoter selected from the group consisting of the xanthate, dithiophosphoric acids and dithiophosphate types, the improvement which comprises carrying out the separation in the presence of 0.01-0.50 lbs. per ton of a surface-modifying agent which comprises a salt of a lignin sulfonate.

2. In the beneficiation by froth flotation of a metallic sulfide mineral by means of a promoter selected from the group consisting of the xanthate, dithiophosphoric acids and dithiophosphate types, the improvement which comprises carrying out the separation in the presence of 0.01-0.50 lbs. per ton of a surface-modifying agent for the metal sulfide mineral which agent comprises a salt of a lignin sulfonate.

3. In the beneficiation by froth flotation of a metallic sulfide mineral from a feed comprising a plurality thereof by means of a promoter selected from the group consisting of the xanthate, dithiophosphoric acids and dithiophosphate types,

15 the improvement which comprises carrying out the separation in the presence of 0.01-0.50 lbs. per ton of a surface-modifying agent for at least one of the metal sulfide minerals, which agent comprises a salt of a lignin sulfonate.

20

ROBERT B. BOOTH.  
ROY A. PICKENS.

25

## REFERENCES CITED

The following references are of record in the 40 file of this patent:

## UNITED STATES PATENTS

| Number    | Name      | Date           |
|-----------|-----------|----------------|
| 2,130,574 | Breerwood | Sept. 20, 1938 |
| 2,238,439 | Bishop    | Apr. 15, 1941  |
| 2,355,365 | Cole      | Aug. 8, 1944   |
| 2,407,651 | Clemmer   | Sept. 17, 1946 |